

[54] METHOD FOR TEXTURIZING  
CONTINUOUS FILAMENTS[75] Inventors: **Hsin L. Li, Parsippany; Hendrikus J. Oswald, Morristown; Alfred L. Liland, Lake Shawnee, all of N.J.**[73] Assignee: **Allied Corporation, Morris Township, Morris County, N.J.**

[\*] Notice: The portion of the term of this patent subsequent to May 24, 1994 has been disclaimed.

[21] Appl. No.: 448,470

[22] Filed: Dec. 10, 1982

## Related U.S. Application Data

[60] Continuation of Ser. No. 250,343, Apr. 2, 1981, abandoned, which is a division of Ser. No. 1,618, Jan. 8, 1979, Pat. No. 4,296,535, which is a continuation-in-part of Ser. No. 799,066, May 20, 1977, Pat. No. 4,133,087, which is a continuation-in-part of Ser. No. 619,085, Oct. 2, 1975, Pat. No. 4,024,611.

[51] Int. Cl.<sup>3</sup> ..... D02G 1/12; D02G 1/16

[52] U.S. Cl. ..... 28/257

[58] Field of Search ..... 28/254, 255, 256, 257

## [56] References Cited

## U.S. PATENT DOCUMENTS

- |           |         |              |          |
|-----------|---------|--------------|----------|
| 3,156,028 | 11/1964 | Weiss et al. | 28/257   |
| 3,526,024 | 9/1970  | Fay          | 28/257 X |
| 3,800,374 | 4/1974  | Ozawa et al. | 28/257   |
| 3,816,887 | 6/1974  | Smith et al. | 28/256   |

|           |        |              |          |
|-----------|--------|--------------|----------|
| 4,019,228 | 4/1977 | Ozawa et al. | 28/257 X |
| 4,024,610 | 5/1977 | Li et al.    | 28/257   |
| 4,024,611 | 5/1977 | Li et al.    | 28/257   |
| 4,040,154 | 8/1977 | Riley        | 28/257   |
| 4,074,405 | 2/1978 | Li et al.    | 28/257   |
| 4,133,087 | 1/1979 | Li et al.    | 28/257   |
| 4,135,280 | 1/1979 | Li et al.    | 28/257   |

## FOREIGN PATENT DOCUMENTS

|          |        |       |        |
|----------|--------|-------|--------|
| 47-17736 | 5/1972 | Japan | 28/257 |
| 51-2533  | 1/1976 | Japan | 28/257 |

Primary Examiner—Robert Mackey

Attorney, Agent, or Firm—Ernest D. Buff

[57]

## ABSTRACT

Continuous filaments are fed into a heating zone. The filaments are then contacted with a stream of heated fluid to increase the temperature of the filaments. The stream of fluid containing the filaments is directed into contact with a barrier disposed within a chamber at a force sufficient to initiate crimping of the filaments. A major portion of the fluid is separated from the filaments and expelled from the chamber. The filaments are transported through the chamber by continuous movement of a surface therein at sufficient velocity to cause overfeeding of the filaments, whereby the filaments are forced against a mass thereof producing crimps therein. One or more streams of heated fluid are then contacted with the mass of filaments to set the crimps. The crimped filaments emerge from the chamber through an outlet opening therein.

9 Claims, 10 Drawing Figures





3  
—  
E — G.



FIG. 4



FIG. 5





FIG. 6







FIG. 10



## METHOD FOR TEXTURIZING CONTINUOUS FILAMENTS

### CROSS-REFERENCE TO RELATED APPLICATIONS

This application is a continuation of application Ser. No. 250,343, filed Apr. 2, 1981 now abandoned; which, in turn, is a division of application Ser. No.: 001,618, filed Jan. 8, 1979, now U.S. Pat. No. 4,296,535 granted Oct. 27, 1981; which, in turn, is a continuation-in-part of application Ser. No.: 799,066, filed May 20, 1977, now U.S. Pat. No. 4,133,087 granted Jan. 9, 1979; which, in turn, is a continuation-in-part of application Ser. No.: 619,085, filed Oct. 2, 1975, now U.S. Pat. No. 4,024,611 granted May 24, 1977 entitled "Method and Apparatus for Texturizing Continuous Filaments."

### BACKGROUND OF THE INVENTION

#### 1. Field of the Invention

This invention relates to method and apparatus for preparing crimped fibrous structures and more particularly to means for crimping textile fibrous materials such as filaments, yarn, tow for staple fibers and the like.

#### 2. Description of the Prior Art

In the apparatus conventionally used to crimp textile strands to increase their bulkiness, a tow of continuous filaments is forced by fluid energy against a mass of tow within a chamber, and emerges in crimped form from the chamber when the pressure on the mass exceeds a certain limit. The number of crimps produced by such apparatus per inch of the filaments, as well as the skein shrinkage or crimp contraction level produced in the filaments, is too low for economical processing of the filaments into high quality knitting yarns, fabrics, high stretch yarns and the like. Higher fluid temperatures, as in the order of 400° C., increase crimping levels but decrease orientation of the filaments, reducing their tensile strength and/or dyeing uniformity. Increasing mass flow of the fluid to heat the yarn at lower fluid temperatures produces turbulence within the chamber, destroying incipient crimp and decreasing the skein shrinkage level of the filaments.

### SUMMARY OF THE INVENTION

The present invention provides a method and apparatus whereby continuous filaments are crimped at relatively low temperature in an economical and highly reliable manner. The filaments, which may be in the form of yarn, are fed into a heating zone, the temperature of the heating zone being, for example, about 100° to 350° C. The filaments are then contacted with at least one stream of heated fluid having a temperature of about 180° to 280° C. to increase the temperature of the filaments and minimize the temperature gradient thereof. The combined stream of fluid and filaments is directed into contact with barrier means disposed within a chamber, the force of contact being sufficient to initiate crimping of the filaments. Upon contact with the barrier means, the major portion of the compressible fluid is separated from the filaments and expelled from the chamber. The filaments are transported through the chamber by continuous movement of a surface therein at sufficient velocity to cause overfeeding of the filaments into the chamber. Due to such overfeeding, the filaments are forced against a mass of the filaments within a zone of compaction in the chamber, producing

crimps therein. One or more streams of heated fluid are then contacted with the mass of filaments to set the crimps. The chamber has an inlet opening for receiving the filaments, fluid jet heating means for contacting the mass with heated fluid and fluid escape means for separating the fluid from the filaments and expelling it from the chamber. A carrier means associated with the chamber forms the continuously moving surface.

It has been found that contacting previously heated filaments with at least one stream of fluid to raise the temperature of the center and exterior surface of each of the filaments in a uniform manner increases the number of crimps per inch of the filaments as well the memory thereof. Further, the flexibility of the filaments is also increased and crimp sharpness is improved. Due to the increased flexibility and crimp sharpness created in the filaments during crimping, the pressure and temperature of the fluids required for crimping are surprisingly low, i.e., about 10 to 500 psig. and about 150° to 350° C. Subsequently contacting the mass of filaments with heated fluid to set the crimps therein further increases filament flexibility and crimp sharpness, the number of crimps per inch of the filaments, and the memory thereof, with the result that the crimps are produced in a highly efficient manner. Crimping levels are unusually high, i.e., in excess of 40 crimps per inch and typically as high as 50 crimps per inch or more. Filament degradation is minimized, skein shrinkage level is greatly improved, i.e., in excess of 35 percent, and uniformity and consistency of crimp are easily controlled. Thus the texturized filaments of this invention permit production of high-bulk and stretch knitting yarn at higher speeds and lower temperatures and costs than those incurred by conventional operations wherein the filaments are crimped using a single heating stage.

### BRIEF DESCRIPTION OF THE DRAWINGS

The invention will be more fully understood and further advantages will become apparent when reference is made to the following detailed description and the accompanying drawings in which:

FIG. 1 is a perspective view illustrating one form of apparatus for contacting previously heated filaments with plural streams of heated fluid, the cover and chamber of the apparatus having a disengaged position and the chamber being partially broken away to show the construction thereof;

FIG. 2 is a section taken along the line 2—2 of FIG. 1, the cover and chamber of the apparatus having a disengaged position;

FIG. 3 is a plan view of another form of apparatus for crimping continuous filaments;

FIG. 4 is a cross-section taken along the line 4—4 of FIG. 3;

FIG. 5 is a perspective view illustrating one form of apparatus for carrying out the method of this invention;

FIG. 6 is a perspective view illustrating another embodiment of the apparatus of FIG. 1.

FIGS. 7-10 are sections illustrating alternative forms of the heating zone used in the apparatus shown in FIG. 1.

### DESCRIPTION OF THE PREFERRED EMBODIMENT

The crimping apparatus of this invention comprises a chamber having inlet, outlet, heating and fluid escape means. Such chamber may be fabricated in a number of

diverse sizes and configurations. For illustrative purposes the invention is described in connection with a chamber having an arcuate configuration. It will be readily appreciated, however, that chambers having linear as well as curvilinear configurations fall within the scope of the present invention.

Referring to FIGS. 1 and 2 of the drawings, crimping apparatus used to contact previously heated filaments with one or more streams of heated fluid is shown generally at 10. The apparatus 10 has a chamber 12 including an inlet opening 14 for receiving the filaments 16 to be crimped and a barrier means 20 which represents a portion of a perforated plate 17, as shown in FIG. 2 and described hereinafter, is disposed within the chamber 12 adjacent inlet opening 14. Continuous filaments 16, preferably in the form of yarn having a temperature of about 15° to 32° C. enter inlet 22 of a heating means, shown generally at 24. Steam or some other heated fluid, such as heated air, nitrogen, carbon dioxide and the like, having a temperature of about 150° to 350° C., preferably about 200° to 330° C., enters fluid inlet 28 and forces filaments 16 along tube 30 of heating means 24. Tube 30 is provided with a second fluid inlet 31 and preferably a plurality of additional fluid inlets for directing at least a second stream of heated fluid, having a temperature of about 150° to 350° C., preferably about 200° to 330° C., into contact with filaments 16 in tube 30 and, optionally, in tube 35 of fluid directing means, shown generally at 37, to increase the temperature of the filaments and minimize the temperature gradient thereof. After contact with streams of fluid 26 and 33, filaments 16 from tube 30 are aspirated into tube 35 of fluid directing means by stream 33 of nozzle 101 and are directed thereby into contact with barrier means 20, the contact having sufficient force to initiate crimping of the filaments 16. Upon contact with barrier means 20, the major portion of the fluid passes through fluid escape means 32 and is thereby separated from the filaments 16 and expelled from the chamber 12. In order to prevent removal of crimp or deformation initiated in the filaments 16 during separation of the fluid therefrom, it is necessary to prevent the filaments from being subjected to tension or drag during the period of their residence in chamber 12. The initially crimped filaments 16 containing incipient crimps are therefore transported through the chamber 12 by a carrier means which comprises a surface 36 formed by screen 17 adapted for movement relative to the chamber 12 at a velocity sufficient to cause overfeeding of the filaments thereinto. Due to such overfeeding the filaments 16 are forced against a mass 38 of the filaments 16 within a zone of compaction 40 (shown in FIG. 3) in the chamber 12 producing crimps therein.

As shown in FIGS. 3 and 5, the apparatus 100 is provided with a crimp setting means, generally indicated at 76, including fluid jet heating means 80, disposed in chamber 12 downstream of fluid directing means 37, for contacting the mass 38 of filaments 16 with a stream of heated fluid from heating vessel 78 to set the crimps therein. The crimped filaments emerge through outlet opening 18 of the chamber 12 in final crimped form.

Chamber 12 is defined by peripheral recess 42 (shown in FIG. 2) in drum 44 and opposing wall 39 of cover 34. The drum 44 is mounted on shaft 46 for rotation about axis x—x. Fluid from nozzle 101 and filaments 16, directed through tube 35 into contact with barrier means 20 disposed in chamber 12, is separated from the fila-

ments 16 and expelled from chamber 12 through passageways 56 formed in drum 44. Drum 44 is provided with discharge ports (not shown) extending through the drum and connecting with an annular chamber 56 under recess 42. The annular chamber 56 is separated from the recess 42 by perforated plate or screen 17, which forms the bottom of recess 42 and, together with chamber 56 and the discharge ports, comprises the fluid escape means 32. Screen 17 has a mesh size ranging from about 50 to 400, and preferably from about 90 to 325.

The barrier means 20 comprises a portion of perforated plate 17 adapted to intercept the compressible fluid stream from fluid directing means 37. In the apparatus shown in FIG. 1 of the drawing, the portion of screen 17 which represents barrier means 20 changes continuously as the periphery of drum 44 rotates. Alternatively, the barrier means can comprise a porous or nonporous plate (not shown) alone or in combination with screen 17, the plate being fixedly mounted on the fluid directing means 37 and projecting to a point of interception with streams 26, 33 inside chamber 12 and adjacent to inlet opening 14 thereof.

Fluid directing means 37 is positioned relative to drum 44 so that the end 48 of tube 35 is in relatively close proximity to barrier means 20. The distance between end 48 and barrier means 20, as well as the cross-sectional area of the end 48 can be varied depending on the velocity and temperature of the filaments and of the fluid stream, the denier of the filaments, the angle at which the stream intersects the barrier means 20, the coefficient of friction of the impacting surface of barrier means 20 and the cross-sectional area of chamber 12. Generally, upon impact with the barrier means 20, fluid streams 26, 33 have a velocity of about 300 to 1,500 feet per second and a temperature of about 100° to 280° C. and a total pressure of about 10 to 500 psig.; and filaments 16 have a velocity of about 200 to 30,000 feet per minute, a temperature of about 100° to 250° C., and a denier of about 1 to 25 per filament, and a yarn denier of about 15 to 5,000. The coefficient of friction of the impacting surface is about 0.05 to 0.9, the angle of impact,  $\theta$ , is about 15° to 75°. The distance between end 48 and point of impact of fluid streams 26, 33 on surface 36 is about 0.01 to 0.5 inch, the cross-sectional area of end 48 is about 0.0002 to 0.75 square inch and the cross-sectional area of chamber 12 is about 0.00015 to 1.00 square inch.

Preferably, fluid streams 26, 33 contact the impacting surface of barrier means 20 at a velocity of about 600 to 1,500 feet per second, a total pressure of about 20 to 300 psig. and a temperature of 180° to 280° C., causing filaments having a denier of about 2 to 15 per filament and a yarn denier of about 21 to 2,600 to contact the impacting surface at a velocity of about 3,000 to 30,000 feet per minute and temperature of about 150° to 220° C. The coefficient of friction of the impacting surface is preferably about 0.1 to 0.6, the angle of impact,  $\theta$ , is preferably about 30° to 70°, the distance between end 48 and point of impact of fluid streams 26, 33 on surface 36 is preferably about 0.02 inch to 0.30 inch, the cross-sectional area of end 48 is about 0.0006 to 0.40 square inch and the cross-sectional area of chamber 12 is about 0.00075 to 0.40 square inch.

Fluid escape means 32 is located with respect to barrier means 20 so that a major portion of fluid streams 26, 33 contacting barrier means 20 is separated from filaments 16 and expelled from chamber 12. The fluid escape means 32 comprises perforated plate or screen 17,

together with exhaust chamber 56 and discharge ports leading to a point exterior of drum 44. The number and diameters of the apertures is sufficient to separate from filaments 16 and expel from chamber 12 a major portion of fluid streams 26, 33 contacting barrier means 20 as in the order of about 60 to 98 percent, and preferably about 70 to 95 percent thereof. The fluid escape means can also comprise a plurality of apertures provided in cover 34.

Referring again to FIGS. 1 and 2, filaments 16 entering compaction zone 40 (shown in FIG. 3) impinge against previously advanced filaments (mass 38 of filaments 16) which has not been withdrawn due to the greater feed rate of filaments 16 into zone 40 in comparison to the rate at which the filaments are removed from the zone. As a result of this overfeed further crimp is imparted to the filaments 16.

After impinging against the mass 38 of filaments 16, the crimped filaments move in recess 42 for about  $\frac{1}{4}$  to  $\frac{1}{2}$  of a rotation of drum 44 during which time they are contacted with a stream of heated fluid from heating vessel 78 (shown in FIG. 3) to set the crimps. Thereafter, the filaments are moved to outlet opening 18 where they are taken up on conventional bobbins using conventional winders and the like. Rear extension block 54 connected to cover 34 by rivets (not shown), adhesive or the like, prevents filaments 16 or plugs thereof, which are inadvertently broken during residence in chamber 12 from re-entering the chamber 12.

The crimp setting means can comprise a fluid jet heating means 80, including at least one passageway 82, and preferably several passageways 82, 83, 85, disposed in cover 34 for communication with chamber 12 downstream of inlet opening 14. Heat of fluid entering vessel 78 travels through passageway 82 into chamber 12 in the form of a stream. The passageway 82 is positioned in cover 34 so that the stream of heated fluid enters the compaction zone 40 contacting the mass 38 of filaments 16 and setting the crimps therein. The temperature, volume, velocity and pressure of the stream of fluid from vessel 78 can vary depending on the denier of the filaments, the cross-sectional area of chamber 12, the rotational velocity of drum 44 and the angle at which the stream intersects the mass 38 of filaments 16. For relatively high speed yarn production, the cross-sectional area of the end 49 of the passageway 82 of the fluid jet heating means 80 should be about 0.0001 to 0.04 square inch, and preferably about 0.0006 to 0.03 square inch. Generally, upon contact with the mass 38 of filaments 16, the stream of fluid has a velocity of about 500 to 1,500 feet per second and a temperature of about 150° to 350° C. and a total pressure of about 5 to 500 psig.; mass 38 has a velocity of about 10 to 5,000 feet per minute, a temperature of about 100° to 220° C., a denier of about 1 to 25 per filament, and a yarn denier of about 15 to 5,000; the cross-sectional area of chamber 12 is about 0.00015 to 1.00 square inch. Preferably, fluid from vessel 78 contacts the mass 38 of filaments 16 at a velocity of about 600 to 1,500 feet per second, a total pressure of about 10 to 300 psig. and a temperature of about 170° to 330° C., setting the crimps in filaments having a denier of about 2 to 15 per filament and a yarn denier of about 21 to 2,600. The angle of impact,  $\phi$ , between the stream of fluid from vessel 78 and mass 38 is preferably about 45° to 135°, and the cross-sectional area of chamber 12 is about 0.00075 to 0.40 square inch.

In the embodiment shown in FIGS. 1, 2 and 5, the carrier means for transporting filaments 16 through

chamber 12 is a surface including walls 50, 52 and perforated plate 17 of recess 42. The carrier means can alternatively be comprised of perforated plate 17 solely. Carrier velocity varies inversely with the surface area thereof and the crimp frequency desired. Generally, the velocity of the carrier means shown in FIGS. 1, 2 and 5 is about 0.1 to 10 percent of the velocity of filaments 16. By varying the velocity of the carrier means, the residence time of filaments 16 in compaction zone 40 is controlled to produce uniformity of crimp and degree of set in the filaments 16 over a wide range of crimp level.

The apparatus 100 which has been disclosed herein can be modified in numerous ways without departing from the scope of the invention. As previously noted, the configuration of chamber 12 can be linear or curvilinear. Barrier means 20 can be porous or nonporous and can comprise a stationary noncontinuous or movable continuous impacting surface. Each of peripheral recess 42 of drum 44 and cover 34 can be perforated to provide for escape of compressible fluid through all sides of chamber 12. The length,  $l$ , of tube 30 can be varied to alter the residence time of filaments 16 therein. Generally, the heating means 24 includes a tube 30 having a length of about 3 to 60 inches; fluid inlets 28, 31 are spaced longitudinally of tube 30 by a center-to-center distance of about 1 to 10 inches; the cross-sectional areas of the fluid inlets 28, 31 are about 0.00008 to 0.03 square inch; and the number of fluid inlets 28, 33 is about 1 to 60. Preferably, tube 30 of heating means 24 has a length,  $l$ , of about 6 to 42 inches; fluid inlets 28, 31 are spaced longitudinally of tube 30 by a center-to-center distance of about 2 to 5 inches; the cross-sectional areas of the fluid inlets 28, 31 are about 0.0003 to 0.020 square inch; the number of fluid inlets 28, 31 are about 2 to 10. The fluid of which streams 26, 33 are comprised can be either compressible or incompressible. Compressible fluids which are suitable include air, steam, nitrogen, argon, gas mixtures and the like. Incompressible fluids which are suitable include water, saturated steam, mixtures of liquids and the like. The heating zone can comprise a stationary heating block(s), a rotating heating roll(s) heated electrically or by high temperature fluids, or one or more infrared, induction or microwave heaters, or a combination thereof, such combination being employed alternatively to or collectively with tube 30 of heating means 24.

As shown in FIGS. 3 and 4, barrier means 20 can be a screen 58 forming a wall of recess 42 in drum 44 opposite wall 60 of cover 34. The drum 44 is mounted on shaft 62' which rotates on bearings (not shown) about axis x—x. Filaments 16 enter tube 62 of a heating means (shown generally at 64). A first stream of heated fluid 49 enters tube 62 through fluid inlet 65 forcing filaments 16 along the tube 62. At least a second stream of heated fluid 66 enters tube 62 through fluid inlets 68 contacting filaments 16 and increasing the temperature thereof. The combined streams of fluid 49, 66 and filaments 16 enter tube 70 of fluid directing means, shown generally at 72. The latter directs the filaments 16 into contact with barrier means 20 disposed in chamber 12 in the manner set forth in connection with FIGS. 1 and 2. Fluid 49, 66 is separated from filaments 16 and expelled from chamber 12 through discharge ports (not shown) connected with passageway 59 of drum 44, as well as through passageway 74 formed between drum 44 and cover 34. A major portion of the fluid 49, 66 can, optionally, be expelled from tube 62 of heating means 64

prior to entering tube 70 of fluid directing means 72, and from chamber 12 through screen 58. The filaments 16 are contacted with one or more streams of heated fluid from vessel 78 (FIGS. 3 and 5) and emerge from chamber 12 through an outlet opening 18 in the manner set forth above in connection with FIGS. 1, 2 and 5.

In FIG. 7, there is shown an embodiment of the invention in which the heating means comprises a stationary heating block 204. Yarn 201 pulled off bobbin 202 is directed through yarn guide 203. Upon movement over stationary heating block 204, the yarn 201 is heated by contact therewith. Thereafter the yarn 201 is aspirated into tube 62 and/or tube 70 and processed in the manner described above in connection with FIGS. 3 and 4. The temperature of block 204 typically ranges from about 150° to 350° C.

In FIG. 8, there is shown an embodiment of the invention in which the heating means is a rotating heating roll 208. Yarn 201 pulled off bobbin 202 is directed through yarn guide 203 by a rotating induction heated roll 208. The yarn 201 is wrapped around the roll 208 nominally 10-20 times while being separated on the roll 208 surface in an axial direction. Separation of yarn 201 on roll 208 is accomplished by use of a yarn separator roll 209, which is a free wheeling cylinder mounted on an axis slightly skewed from that of roll 208 and outside the cylindrical surface bounded by roll 208. The roll 208 is heated by stationary induction heating coils (not shown). Generally, the temperature of the induction coils ranges from about 100° to 300° C.

FIG. 9 illustrates an embodiment of the invention in which the heating means comprises an infrared heater. Yarn 201 from bobbin 202 is directed through yarn guide 203. Thereafter, the yarn 201 passes through infrared oven 210 which contains quartz heating rods 211. These rods 211 heat the moving yarn by infrared radiation. The yarn 201 is then aspirated into tube 62 and/or tube 70 and processed in the manner described in connection with FIGS. 3 and 4. Generally, the temperature of heating rods 211 ranges from about 500° to 1200° C.

FIG. 10 depicts an embodiment of the invention wherein the heating means comprises the combination of an induction heater 212 and a stationary heating block 204. Yarn containing metallic fillers 215 is pulled from bobbin 202 and directed through yarn guide 203. The yarn 215 then passes through induction heater 212 having at least one inductor coil 213. Inductor coil 213 carries a high-frequency, alternating current which creates eddy currents in the metallic filler, thereby generating heat in the yarn 215. The yarn 215 is thereafter guided over stationary heating block 204 and processed in the manner described above with reference to FIGS. 3 and 4. Generally, the frequency of the inductor coil ranges from about 1 KHz to 6 KHz and the surface temperature of block 204 adapted for contact with yarn 215 ranges from about 200° to 300° C.

In operation, yarn in the form of continuous filaments 16 is fed by aspiration into a heating zone. The filaments are thereafter contacted with at least one stream 49, 66 of fluid to increase the temperature thereof in a uniform manner. Fluid directing means 72 directs the stream of fluid 49, 66 containing filaments 16 into contact with barrier means 20, disposed within chamber 12, to initiate crimping of the filaments 16. Fluid escape means 32 separates the major portion of the fluid from the filaments 16 and expels it from chamber 12. A carrier means transports the filaments 16 through chamber 12 to cause overfeeding of the filaments 16 into the cham-

ber. One or more streams of heated fluid are directed by fluid jet heating means 80 into contact with the mass 38 of filaments 16 to set the crimps. The filaments emerge from the chamber 12 in crimped form and are wound onto packages.

As shown in FIG. 6, tube 30 can be angularly positioned relative to tube 35 to facilitate separation of fluid from the filaments 16, the latter being directed into tube 35 by heated fluid from nozzle 101. These and other modifications are intended to fall within the scope of the invention as defined by the subjoined claims.

While the method and apparatus of this invention have been described herein primarily in terms of texturizing thermoplastic filaments, especially polyester filaments, it is clear that the method and apparatus of the present invention can also be used to crimp a wide variety of other filaments, such as filaments composed of homopolymers and copolymers of the following materials: poly  $\epsilon$ -aminocaproic acid, hexamethylene adipamide, ethylene terephthalate, tetramethylene terephthalate, 1,4-cyclohexylenedimethylene terephthalate and blends thereof. In addition, the filaments 16 can be composed of polyacrylonitrile, polypropylene, poly-4-aminobutyric acid, cellulose acetate and blends thereof.

The following example is presented in order to provide a more complete understanding of the invention. The specific techniques, conditions, materials and reported data set forth to illustrate the principles and practice of the invention are exemplary and should not be construed as limiting the scope of the invention.

#### EXAMPLE 1

Polyethylene terephthalate chips having a number average molecular weight of 25,000 were melt spun using a screw type extruder in which the barrel and dye temperatures were maintained at 270° C. and 280° C., respectively. The spinnerette used had 34 holes, each hole having a capillary diameter of 0.010 inch and a length of 0.010 inch. An air quenched system was used to solidify the filaments. The yarn was a 255 denier, 34 filament, zero twist, partially oriented yarn having a round cross-section. The yarn was coated with approximately 0.25% by weight of a textile finish agent and drawn using a draw ratio of 1.9. The drawing process consisted of passing 10 wraps of the yarn around (1) a pair of heated rolls maintained at a temperature of 75° C., (2) a stationary block heater 6 inches long having a temperature of 180° C., and (3) a pair of draw rolls having a temperature of 175° C. The final drawn denier was 134. Drawing speed was 4,500 feet per minute.

The yarn was textured using the apparatus shown generally in FIGS. 3 and 5. Nozzle 101 had a diameter,  $d$ , of 0.062 inch and a length,  $l$ , of 0.125 inch. Superheated steam at 325° C. and 100 psig. was supplied into nozzle 101 through conduit means (not shown). Heating means 24 included (1) a tube 30 having a length of 20 inches, an average inside diameter of 0.080 inch and an outside diameter of 0.150 inch, and (2) a fluid inlet having an inside diameter of 0.036 inch. Steam under pressure of 80 psig. flowed through the fluid inlet into tube 30 forcing filaments 16 therethrough. The filaments then entered energy tube 35 and were carried at 8,300 feet per minute therethrough and into contact with barrier means 20. Energy tube 35 had an inside diameter of 0.101 inch, and was 5 inches long. The yarn was heated to a temperature of about 160° C. during residence in energy tube 35 and impinged against barrier means 20 at an impact angle,  $\theta$ , of 60°. The barrier

means 20 was a perforated brass plate 17, 10 inches in diameter and spaced 0.030 inch from the exit orifice 48 of energy tube 35. The perforated brass plate 17 had a thickness of 0.013 inch, a hole-diameter of 0.012 inch and a center-to-center distance between adjacent holes of 0.016 inch, providing the plate with 42% open area. Chamber 12 had a width of 0.200 inch and a depth of 0.030 inch. Chamber 12 was rotated at 25 rpm to provide plate 17 with a surface speed of 65.4 feet per minute. Contact between the yarn containing stream and the plate 17 initiated crimping of the filaments 16. Perforated plate 17 transported the yarn to a zone of compaction 40 wherein a textured plug was formed causing further crimping of the filaments 16. The packing density of the textured plug was calculated to be 33% and the residence time of the plug in chamber 12 was 0.91 seconds. Fluid jet heating means 80 included five passageways disposed in cover 34 in communication with chamber 12. Each of the passageways had an internal diameter of 0.027 inches. The passageways were 20 equally spaced 1.5 inch apart circumferentially of cover 34 commencing 5.5 inches downstream of the end of fluid directing means 35. Steam supplied to the passageways by vessel 78 contacted mass 38 of filaments 16 at a pressure of 18 psig. and a temperature of 138° C. 25

The yarn emerged in crimped form from the chamber through outlet opening 18 and was taken up onto conventional parallel wound packages rotated on conventional winders by means of a pair of rollers (not shown). The speed of the winder was approximately 6,850 feet 30 per minute.

The average skein shrinkage level of the textured yarn was then determined. The skein shrinkage test consisted of winding the textured yarn into a skein and hanging the skein under no load in a hot air oven at 145° 35 C. for 5 minutes. The skein was removed from the oven and cooled, and a 0.0016 gram per denier weight was hung on it. The new skein length was measured ( $L_f$ ). The percent of skein shrinkage was then calculated from the initial skein length ( $L_o$ ) and the final skein 40 length ( $L_f$ ) in accordance with the equation  $(L_o - L_f)/L_o$ . Photomicrographs made of 20 filaments selected at random from the textured yarn showed a crimp count of about 40 crimps per inch. The developed skein had an average skein shrinkage level of 36 percent, indicating 45 that the texture yarn was suitable for use in manufacture of wearing apparel.

The textured yarn produced in accordance with Example 1 was knitted on a Lawson-Hemphill Fiber Analysis knitter having a 54 gauge head, 220 needles, a diameter of 3.5 inches and 36 inches per course. The knitted fabric, when dyed, showed good uniformity and was 50 free from streaks. In addition, the fabric had a soft texture, dimensional stability and pleasing appearance.

Having thus described the invention in rather full detail, it will be understood that these details need not be strictly adhered to but that various changes and modifications may suggest themselves to one skilled in the art. It is accordingly intended that all matter contained in the above description and shown in the accom- 60

panying drawings shall be interpreted as illustrative and not in a limiting sense.

What we claim is:

1. A method of crimping continuous filaments, comprising the steps of:

- (a) heating said filaments in a heating zone;
- (b) feeding said filaments into a heating means having an inlet tube in close communication with a chamber having a stationary cover;
- (c) contacting said filaments with at least one stream of heated fluid within said heating means to increase the temperature of the filaments;
- (d) directing said stream containing said filaments into contact with barrier means disposed within the chamber, the contact occurring at an angle from 15° to 75° and having sufficient force to initiate crimping of said filaments;
- (e) separating a major portion of said stream of heated fluid from said filaments and expelling it from said chamber;
- (f) transporting said filaments through said chamber by continuous movement of a surface therein at sufficient velocity to cause overfeeding of said filaments into said chamber, said filaments being forced against a mass thereof within said chamber to produce crimps therein;
- (g) contacting said mass with at least one stream of heated fluid to set the crimps;
- (h) removing said filaments in crimped form from said chamber; and
- (i) preventing broken filaments or plugs thereof from reentering said chamber, after moving to and emerging from the outlet opening thereof, with a rear extension affixed to said cover to the rear of said inlet tube.

2. A method as recited in claim 1, wherein said filaments contact said barrier means at a velocity of about 3,000 to 30,000 feet per minute.

3. A method as recited in claim 1, wherein said streams of fluid are compressible.

4. A method as recited in claim 1, wherein the number of streams of fluid contacting said filaments is about 1 to 60.

5. A method as recited in claim 1, wherein the mass is contacted with a plurality of streams of fluid.

6. A method as recited in claim 1, wherein said stream of fluid has a temperature of about 150° to 300° C.

7. A method as recited in claim 1, wherein said filaments are composed of polyester.

8. A method as recited in claim 1, wherein said filaments are composed of material selected from the group consisting of poly 1,4-cyclohexylenedimethylene terephthalate, polyethylene terephthalate, polyhexamethylene adipamide, poly ε-aminocaproic acid, polypropylene cellulose acetate, cellulose tri-acetate and blends thereof.

9. A method as recited in claim 1, wherein said filaments are composed of polyamide.

\* \* \* \* \*